

# UNITED STATES PATENT OFFICE.

CARLETON ELLIS, OF LARCHMONT, NEW YORK, ASSIGNOR, BY MESNE ASSIGNMENTS,  
TO COPPER OIL PRODUCTS COMPANY, A CORPORATION OF NEW YORK.

## WOOD-COATING COMPOSITION.

1,005,623.

Specification of Letters Patent. Patented Oct. 10, 1911.

No Drawing.

Application filed May 7, 1909. Serial No. 494,701.

*To all whom it may concern:*

Be it known that I, CARLETON ELLIS, citizen of the United States, residing at Larchmont, in the county of Westchester and State 5 of New York, have invented certain new and useful Improvements in Wood-Coating Composition, of which the following is a specification.

This invention relates to shingle stains 10 and relates particularly to shingle stain compositions carrying oil-soluble metallic compounds or metallo-organic compounds such as copper oleate in solution in oils having siccative properties.

15 Heretofore it has been the custom to make use of creosote to a large extent in the manufacture of shingle stains often in conjunction with sufficient linseed oil to give the composition drying properties. A good 20 many difficulties have arisen in connection with the practical application of such a shingle stain. The action of creosote or similar carbolic acid material on many pigments is pronounced and after the wood has 25 been impregnated with creosote, it is difficult to so apply a coat of ordinary paint as to secure satisfactory adherence. The creosote frequently acts upon the paint vehicle causing the coating to peel. Then of course 30 the odor of creosote is disagreeable to many. In localities where a great deal of construction work is under way and creosote is being employed from time to time for staining purposes, its unpleasant odor continually 35 pervades the air. Under certain conditions creosote has been found to exert a tendering or weakening action on wood fiber. To overcome the difficulties experienced with creosote, it has been proposed to make use of 40 mixtures of kerosene oil and linseed oil, but without any preservative agent, and of course such mixtures are useful only if temporary effects are required.

45 It is the object of the present invention to make use of an oil composition which is neutral and free from creosote or other harmful or objectionable material and at the same time not open to the objections of the

linseed oil and kerosene mixtures containing no preservative agent. The present invention involves the use of an oil-soluble preservative body, preferably a metallo-organic compound such as copper oleate. 50

While various metallic compounds may be used in the present composition including 55 those of lead, tin, arsenic, zinc and the like, I prefer to employ copper compounds owing to the remarkable fungicidal and bactericidal properties of copper. While creosote is an excellent bactericide, it has only feeble 60 properties as a fungicide, and inasmuch as shingles are often attacked by the fungus known as dry rot, it becomes necessary in preparing a shingle stain composition of extreme permanency and durability to employ a body having pronounced fungicidal properties. In this respect, copper stands 65 preëminent. It does all that creosote will do, as a preservative, and more, as it is specific against the attack of dry rot fungus. 70 With such copper compounds, by the joint use of mineral oils and drying oils, a composition may be made which is practically odorless and which dries in a day. It may be made so penetrative that the surface fibers 75 and even those well below the surface of the shingle, are thoroughly protected against influences of decay. The copper compound has the advantage also of rendering the material rather more water-proof than the creosote mixtures so that the shingles are less affected by moisture. Owing to the possibility of making compounds of entirely neutral character from this material, the objections raised against creosote that it is a 80 corrosive acid and injures the hands and clothing of the workmen do not here obtain. The composition is without corrosive action 85 and not unpleasant to use, and furthermore requires no special skill in its application. 90

A formula illustrative of my invention consists of linseed oil 2 quarts, light mineral oil 1 gallon, kerosene oil 1½ quarts, Japan drier ½ quart, copper oleate 6 ozs. and pigment 8 ozs. 95

A cheaper composition may be made from

linseed oil, 2 quarts, light mineral oil  $1\frac{1}{2}$  gallons, light kerosene oil 2 quarts, Japan drier  $\frac{1}{2}$  quart, copper oleate 6 ozs., using about 12 ozs. pigment or sufficient to give the 5 requisite tint.

If it be desired to have a compound of high flash point, the kerosene may be replaced by light mineral oil as in the following formula; linseed oil 2 quarts, light mineral oil of a specific gravity .865  $1\frac{1}{2}$  gallons, 10 manganese resinate 2 ozs., copper oleate 4 ozs., and sufficient pigment to supply the requisite shade of color.

In using kerosene oil I prefer to employ 15 a grade having a flash point of about  $120^{\circ}$  and a fire point of about  $150^{\circ}$  F. Ordinary Japan drier may be used, such as a solution of resinate of manganese or lead, etc., in turpentine. Mineral oil offers a cheap 20 and convenient carrier for the copper compound and the lighter mineral oils such as spindle oils are the most satisfactory in this respect although I have employed heavier mineral oils such as  $25^{\circ}$  paraffin oil with 25 satisfactory results. Of the drying oils, linseed oil is the most satisfactory owing to its permanency and because of the readiness with which it dissolves the copper compound in the presence of mineral oil. Of 30 course other drying oils may be used to a more or less degree and also semi-drying oils such as corn, cotton seed and rosin oil.

The copper oleate has the distinct advantage over copper resinate, copper carbonate and similar copper compounds of being remarkably soluble in mineral and linseed oil mixtures. It is not an easy matter 35 to incorporate resinate of copper or carbonate of copper in such mixtures to a degree sufficient to secure satisfactory protective 40 qualities, and I have found that through the use of copper oleate, results may be secured which are entirely satisfactory. The copper oleate unlike the resinate is not affected 45 by the changes in temperature nor is it influenced to any great extent by the presence of other metallo-organic bodies or by driers, etc. It is readily made, a satisfactory stock being obtained, for example, by heating copper 50 carbonate or hydrate with commercial oleic acid (known as red oil) to a temperature of  $140^{\circ}$  to  $150^{\circ}$  C. The resulting melt when cold is of a soft waxy consistency and dissolves with the utmost ease in the oils 55 above mentioned, producing a compound which is extremely active and efficient as the copper is actually in solution, and every portion of the oil is therefore highly effective. The case is different where solid and 60 oil-insoluble copper compounds are ground in oil mixtures as in the manufacture of antifouling paints and the like, for the oil-

insoluble copper compounds remain entirely on the surface of the wood and do not penetrate into the fibers to any appreciable extent. Therefore, although the copper in this solid and oil-insoluble form may temporarily exert some protective influence, eventually it chips and flakes away leaving the wood bare and without preservative. 65 On the other hand, with the solution of copper oleate, the wood fibers are impregnated for a considerable distance below the surface with the copper compound, and even though the superficial layer of the pigment become 70 removed in the course of time by weathering and erosion, the wood is still protected by the soluble copper compound which originally penetrated into the fibers of the wood below the surface. It will be evident that 75 the above mixtures of linseed oil, mineral oil and copper oleate are free from offensive odor and in fact such slight linseed or mineral oil odor as the composition may possess, quickly disappears on exposure of the wood. 80 85

A great variety of pigments may be employed in coloring the aforesaid oil to the desired shade, as for example, raw or burnt 90 umber for brown, Indian red, mineral red and the like for red shades, Brunswick green or chrome green or mineral green for 95 green tones, ocher, Indian yellow, chrome yellow and the like for yellow shades, and Prussian blue, lampblack, etc., for blue and black tones. Only a few ozs. of pigment are 95 required per gallon of the composition to give the requisite intensity.

The pigment should be very finely ground and I prefer to mix the pigments with mineral oil instead of linseed oil for the 100 purpose of grinding, passing them through a roll grinder several times in order to reduce the particles of the pigment to the finest possible degree of subdivision so as to permit of the pigment being suspended 105 in the solution for a long period of time after agitation in order that frequent mixing of the composition may not be required during its application. A peculiar and artistic effect may be obtained by the addition 110 of small quantities of neutral powders such as aluminum or copper bronze powders.

In order to get a fire proof composition, I may chlorinate various aromatic oils or compounds such as the light hydrocarbon 115 from coal tar or naphthalene and the like, some of which afford substantially fixed oils of such a degree of chlorination, that they are practically non-inflammable. Such a composition when applied to a shingled roof 120 has a distinct advantage in the case of fire in an adjacent building; for sparks lodging on the roof of a building coated with ordinary shingle stain sometimes quickly start

106. COMPOSITIONS,  
COATING OR PLASTIC.

18

1,005,623

3

fires. With the chlorinated oil as the basis, little danger is to be apprehended from this source.

Having described my invention to the details of which I do not wish to limit myself, what I claim is:—

1. A shingle stain composition comprising copper oleate, a drying oil and a chlorinated compound of naphthalene.
- 10 2. A wood coating composition, comprising

ing copper oleate, a drying oil, and a substantially fixed chlorinated compound of naphthalene.

In testimony whereof I have affixed my signature in presence of two witnesses.

CARLETON ELLIS.

Witnesses:

NATHANIEL L. FOSTER,  
JAMES D. REMSEN.

Copies of this patent may be obtained for five cents each, by addressing the "Commissioner of Patents, Washington, D. C."